

Dwight & Wells

Plow Mold Board

No 90,512.

Patented May 25, 1869.



Inventors,  
S. H. Dwight  
and C. Wells,  
by their Atty.  
H. Howzein

Witnesses,  
Charles Foster  
John Parker

# United States Patent Office.

SOLOMON H. DWIGHT, OF DECATUR, ILLINOIS, AND CALVIN WELLS, OF PITTSBURG, PENNSYLVANIA.

*Letters Patent No. 90,512, dated May 25, 1869.*

## IMPROVED COMPOUND MOULD-BOARD FOR PLOWS.

The Schedule referred to in these Letters Patent and making part of the same.

*To all whom it may concern:*

Be it known that we, SOLOMON H. DWIGHT, of Decatur, Illinois, and CALVIN WELLS, of Pittsburg, Pennsylvania, have invented an Improvement in the Manufacture of Mould-Boards for Plows; and we do hereby declare the following, to be a full, clear, and exact description of the same.

Our invention consists of a mould-board for plows, made of steel, welded between two plates of iron, properly shaped and hardened, and then so ground as to remove the iron from one side and expose a facing of hardened steel, all substantially as described hereafter.

The object of our invention is to produce a perfect, unwarped mould-board, in which all the advantages of both steel and iron are available.

In order to enable others skilled in the art to make our invention, we will now proceed to describe the mode of carrying it into effect, reference being had to the accompanying drawing, which forms a part of this specification, and in which the figure represents sufficient of the mould-board of a plow to illustrate our invention.

Many attempts have been made, in the manufacture of mould-boards for plows, to so combine iron and steel that all the advantages of the latter, as regards strength and hardness, might be rendered available, and its brittle quality counteracted by the more flexible iron.

For instance, a mould-board has been made by welding a facing of steel to an iron backing, but this plan has been found defective, owing to the difficulty of hardening the steel without warping, and sometimes cracking the same—a difficulty owing to want of uni-

son in the contractile properties of the two materials after heating.

This difficulty we overcome by welding the plate A, of steel, between two plates, B and B', of iron. Of this compound plate the mould-board is properly shaped, and then hardened, after which the iron is ground away on one side, so as to leave a smooth, hardened facing of steel properly backed by iron.

During the hardening-process, the steel, protected as it is on both sides by the iron plates, is prevented from warping and cracking during shrinkage, and retains the exact shape imparted to it.

We claim as our invention, and desire to secure by Letters Patent—

A mould-board for plows, made of steel, welded between two plates of iron, then properly shaped and hardened, and afterward so ground as to remove the iron from one side and expose a facing of steel, all substantially as and for the purpose herein set forth.

In testimony whereof, we have signed our names to this specification, in the presence of two subscribing witnesses.

SOLOMON H. DWIGHT.  
CALVIN WELLS.

Witnesses to the signature of S. H. DWIGHT:

HENRY B. DURFEE,  
B. K. DURFEE.

Witnesses to the signature of CALVIN WELLS:

RODOLF ROERNIG,  
HENRY SCHWER.